# EUROPEAN PATENT APPLICATION

(11) **EP 4 782 570 A1**
(43) Date of publication of application: **29.07.2026**
(21) Application number: 23953219.5
(22) Date of filing: 20.12.2023
(51) Int. Cl.: C23C 22/07, C23C 22/82, C23C 22/74, C21D 8/12

(54) **INSULATION COATING COMPOSITION FOR ELECTRICAL STEEL SHEET, ELECTRICAL STEEL SHEET, AND METHOD FOR MANUFACTURING SAME**

(30) Priority: 20.09.2023 KR 20230125559
(71) Applicant: POSCO Co., Ltd, Pohang-si, Gyeongsangbuk-do 37859 (KR)
(72) Inventor: KIM, Hyunjong, Pohang-si, Gyeongsangbuk-do 37859 (KR); NO, Taeyoung, Pohang-si, Gyeongsangbuk-do 37859 (KR)
(74) Representative: Meissner Bolte Partnerschaft mbB
(86) International application number: PCT/KR2023/021092
(87) International publication number: WO 2025/063397

(57) **Abstract**

An insulation coating composition for an electrical steel sheet according to an embodiment of the present disclosure includes: 100 parts by weight of metal phosphate; 25 to 150 parts by weight of silica; 15 to 60 parts by weight of metal oxyhydroxide; and 0.5 to 10 parts by weight of a reducing agent.

## Description

### [Technical Field]

An embodiment of the present disclosure relates to an insulation coating composition for an electrical steel sheet, the electrical steel sheet, and a method for manufacturing the same. Specifically, the present disclosure relates to an insulation coating composition for an electrical steel sheet appropriately combining components of the insulation coating composition to have excellent durability in a high-temperature and high-humidity environment, extreme corrosion resistance, and excellent heat resistance at a very high temperature such as stress relief annealing (SRA), the electrical steel sheet, and a method for manufacturing the same.

### [Background Art]

An electrical steel sheet is a product used as a material for a transformer, a motor, and an electrical device, and unlike a general carbon steel that emphasizes processability such as a mechanical characteristic, the electrical steel sheet is a functional product that emphasizes an electrical characteristic. The electrical characteristic includes low iron loss, high magnetic flux density, high permeability, and a high space factor.

The electrical steel sheet is classified into a grain-oriented electrical steel sheet and a non-oriented electrical steel sheet. The grain-oriented electrical steel sheet is an electrical steel sheet with an excellent magnetic characteristic in a rolling direction by forming Goss structure ({110}<001> texture) throughout the steel sheet using an abnormal grain growth phenomenon called secondary recrystallization. The non-oriented electrical steel sheet is an electrical steel sheet in which a magnetic characteristic is uniform in all directions on a rolled sheet.

Formation of an insulation coating is a process corresponding to a final manufacturing process of a product, and the insulation coating usually requires a good electrical characteristic that suppresses generation of an eddy current, good continuous punching processability that suppresses wear of a mold when it is manufactured as an iron core by being stacked as a plurality of layers after being punched into a predetermined shape, good sticking resistance in which iron core steel sheets do not adhere to each other after stress relief annealing (SRA) that restores a magnetic characteristic by removing processing stress of the steel sheet, good surface adhesion, and the like. In addition to the basic characteristic, excellent application workability of a coating solution and stability of the solution that may be used for a long time after mixing are also required in the insulation coating. The coating solution used for this purpose includes a chromium coating based on chromic acid and a phosphate coating based on phosphate.

The coating has a disadvantage of poor corrosion resistance. Additionally, it is known that various solution properties are inferior if chromium is not added. Therefore, there may be a need to develop an insulation coating that is environmentally friendly and has relatively excellent corrosion resistance.

### [Disclosure]

### [Technical Problem]

An embodiment of the present disclosure provides an insulation coating composition for an electrical steel sheet, the electrical steel sheet, and a method for manufacturing the same. Specifically, the embodiment of the present disclosure provides an insulation coating composition for an electrical steel sheet appropriately combining components of the insulation coating composition to have excellent durability in a high-temperature and high-humidity environment, extreme corrosion resistance, and excellent heat resistance at a very high temperature such as stress relief annealing (SRA), the electrical steel sheet, and a method for manufacturing the same.

### [Technical Solution]

An insulation coating composition for an electrical steel sheet according to an embodiment of the present disclosure includes: 100 parts by weight of metal phosphate; 25 to 150 parts by weight of silica; 15 to 60 parts by weight of metal oxyhydroxide; and 0.5 to 10 parts by weight of a reducing agent.

The metal phosphate may include at least one of Mg, Ca, Ba, Sr, Zn, and Al.

The silica may have a pH of 8 to 12.

The metal oxyhydroxide may include at least one of TiOOH, ZrOOH, and MnOOH.

The reducing agent may include at least one of ammonia, glycol, polyol, and sulfate.

The reducing agent may include at least one of ammonia, ethylene glycol, propane-1,2,3-triol, and sodium sulfate.

An electrical steel sheet according to an embodiment of the present disclosure includes: an electrical steel sheet substrate; and an insulation coating that is disposed on a surface of the electrical steel sheet substrate. The insulation coating includes 100 parts by weight of metal phosphate, 25 to 150 parts by weight of silica, 15 to 60 parts by weight of metal oxyhydroxide, and 0.5 to 10 parts by weight of a reducing agent.

A method for manufacturing the electrical steel sheet according to an embodiment of the present disclosure includes: preparing an electrical steel sheet substrate; applying an insulation coating composition to a surface of the electrical steel sheet substrate; and heat-treating the electrical steel sheet substrate. The insulation coating composition includes 100 parts by weight of metal phosphate, 25 to 150 parts by weight of silica, 15 to 60 parts by weight of metal oxyhydroxide, and 0.5 to 10 parts by weight of a reducing agent.

The heat-treating of the electrical steel sheet substrate may be performed at a temperature of 750 to 1000°C for 10 to 300 seconds.

### [Advantageous Effects]

An embodiment of the present disclosure may have excellent durability in a high-temperature and high-humidity environment, extreme corrosion resistance, and excellent heat resistance at a very high temperature for processability such as stress relief annealing (SRA).

An embodiment of the present disclosure may have a very excellent insulation effect in a high-frequency magnetic field environment.

### [Description of the Drawings]

FIG. 1 is a schematic diagram of a cross-section of an electrical steel sheet according to an embodiment of the present disclosure.

### [Mode for Invention]

Terms such as "first", "second", and "third" are used herein to describe various portions, components, regions, layers, and/or sections, but are not limited thereto. The terms are used only to distinguish one portion, component, region, layer, or section from another portion, component, region, layer, or section. Accordingly, a first portion, component, region, layer, or section described below may be referred to as a second portion, component, region, layer, or section within a scope that does not depart from a scope of the present disclosure.

A technical term used herein is intended only to refer to a specific embodiment, and is not intended to limit the present disclosure. Singular forms used herein also include plural forms unless phrases clearly indicate an opposite meaning. A term "include" used in the specification specifies a specific characteristic, region, integer, step, operation, element, and/or component, and does not exclude presence or addition of another characteristic, region, integer, step, operation, element, and/or component.

When it is said that a portion is "on" or "above" another portion, the portion may be disposed directly on or above the other portion, or another portion may be interposed therebetween. In contrast, when a portion is said to be "directly above" another portion, no other portion is interposed therebetween.

Although not otherwise defined, all terms used herein, including a technical term and a scientific term, have the same meanings as those generally understood by a person of ordinary skill in the art to which the present disclosure belongs. Terms defined in a dictionary commonly used are additionally interpreted to have a meaning consistent with the relevant technical literature and the presently disclosed contents, and are not interpreted in an ideal or very formal sense unless otherwise defined.

Hereinafter, an embodiment of the present disclosure will be described in detail with reference to the accompanying drawings so that a person of ordinary skill in the art to which the present disclosure belongs may easily implement the present disclosure. The present disclosure may be modified in various ways, all without departing from the spirit or scope of the present disclosure.

An insulation coating composition for an electrical steel sheet according to an embodiment of the present disclosure may include 100 parts by weight of metal phosphate, 25 to 150 parts by weight of silica, 15 to 60 parts by weight of metal oxyhydroxide, and 0.5 to 10 parts by weight of a reducing agent.

Hereinafter, each component will be described in detail. In an embodiment of the present disclosure, the parts by weight may mean a relative weight ratio based on 100 parts by weight of the metal phosphate, and may be based on a solid content of each component. The solid content may refer to a weight when each component is dried in a state in which a volatile matter such as a solvent does not exist. For example, it may refer to a weight remaining after heat treatment when a heat treatment process is performed during formation of an insulation coating.

The metal phosphate may serve as a binder within the insulation coating composition. If the metal phosphate is not included in an appropriate amount, adhesiveness of an insulation coating may be deteriorated, or a tension may not be sufficiently obtained. The metal phosphate may be manufactured by a manufacturing process in which metal oxide is added to pure phosphoric acid (H₃PO₄) to react with the pure phosphoric acid (H₃PO₄). In order to improve adhesiveness of the metal phosphate, boric acid may be additionally added during a reaction process and may be maintained for 3 hours or more to induce a condensation reaction between the metal phosphate and the boric acid, and the condensation reactant may be used instead of the metal phosphate. In an embodiment of the present disclosure, the metal phosphate may include not only the metal phosphate but also a condensation reactant of the metal phosphate and the boric acid. The manufactured metal phosphate may exhibit strong acidity.

The metal phosphate may be added to a composition using a solution having a solid content of 50 to 70 wt%. In this case, if the solid content within the solution is too small, free phosphoric acid may be increased within the metal phosphate so that surface moisture absorption occurs after the metal phosphate is manufactured, and if the solid content is too large, a reaction may be poor and precipitation may occur due to an excess of the solid content compared with the pure phosphoric acid.

The metal phosphate and the metal oxide may include various metals without limitation. For example, a metal of each of the metal phosphate and the metal oxide may include one or more of Mg, Ca, Ba, Sr, Zn, and Al. In some embodiments, the metal phosphate may include at least one of monobasic magnesium phosphate (Mg(H₂PO₄)₂) and monobasic aluminum phosphate (Al(H₂PO₄)₃). For example, the metal phosphate may include the monobasic magnesium phosphate (Mg(H₂PO₄)₂) and the monobasic aluminum phosphate (Al(H₂PO₄)₃). In this case, based on a solid content, the metal phosphate may include 10 to 40 parts by weight of the monobasic aluminum phosphate and 60 to 90 parts by weight of the monobasic magnesium phosphate based on a total 100 parts by weight. If too little monobasic aluminum phosphate is included, an effect of improving a tension by adding the monobasic aluminum phosphate may not be sufficient. If too much monobasic aluminum phosphate is added, an Al component may increase crystallization of silica to cause a crack within the insulation coating. For example, based on a solid content, the metal phosphate may include 15 to 35 parts by weight of the monobasic aluminum phosphate and 65 to 85 parts by weight of the monobasic magnesium phosphate or 20 to 30 parts by weight of the monobasic aluminum phosphate and 70 to 80 parts by weight of the monobasic magnesium phosphate based on a total 100 parts by weight.

An insulation coating composition for an electrical steel sheet according to an embodiment of the present disclosure may include 25 to 150 parts by weight of silica based on 100 parts by weight of the metal phosphate.

The silica may be a component necessary to reduce iron loss by providing a tension to the steel sheet. If too little silica is included, it may be difficult to obtain a sufficient effect of applying a tension to the steel sheet. If too much silica is included, a problem may occur in a sticky property or solution stability. For example, the insulation coating composition may include 30 to 130 parts by weight of the silica or 35 to 100 parts by weight of the silica based on 100 parts by weight of the metal phosphate.

The silica may include basicity and acidity, and for example, the silica may include basicity. If the silica includes basicity, stability of the insulation coating composition may be advantageous, and a keeping property of the solution may be improved. Basic silica may have a pH of 8 to 12. The silica may be dispersed in a form of a sol to measure the pH.

The silica may have an average particle diameter in a range of 5 to 20 nm. If the average particle diameter of the silica is too small, a speed of a condensation reaction may be fast so that an agglomeration phenomenon occurs and a color deviation defect is caused on a surface thereof. If the average particle diameter of the silica is too large, a surface area per unit mass may be decreased so that a speed of the condensation reaction is decreased and a defect occurs due to the decreased speed. For example, the silica may have an average particle diameter in a range of 10 to 15 nm. In an embodiment of the present disclosure, a particle diameter may be measured by a particle size measuring device (Zeta Potential), and the average particle diameter may be an arithmetic average.

The silica may include at least one nanoparticle having different average particle diameters. For example, the silica may be used by mixing at least one silica nanoparticle having different average particle diameters to form an insulation coating having an excellent coating characteristic.

An insulation coating composition for an electrical steel sheet according to an embodiment of the present disclosure may include 15 to 60 parts by weight of metal oxyhydroxide based on 100 parts by weight of the metal phosphate. The metal oxyhydroxide may be a compound represented by Mₓ(OOH)_{y}, and M may represent a metal and x and y may represent a ratio according to an oxidation number of the metal. A conventional insulation coating composition may include an oxide particle such as TiO₂, ZrO₂, or MnO₂ as an inorganic ceramic particle. However, in this case, a solution may be gelled so that a problem occurs in stability of the solution. If the metal oxyhydroxide is added to the insulation coating composition as in an embodiment of the present disclosure, the metal oxyhydroxide may be dissolved in the solution in a composition state so that stability of the solution is excellent. During a formation process of the insulation coating, the metal oxyhydroxide may react with a reducing agent to be changed into an insoluble material. That is, if the metal oxyhydroxide is present in the insulation coating composition, a viscosity of the solution may be maintained close to a Newtonian fluid characteristic for application to a natural coater. In some embodiments, a viscosity of the insulation coating composition may be maintained at 10 c.p. or less. For example, the viscosity may be 1 to 10 c.p.. In this case, the viscosity may be measured based on a Brookfield viscometer at a temperature of 30°C.

If too little metal oxyhydroxide is included, a problem of poor weather resistance and poor corrosion resistance of the insulation coating may occur. If too much metal oxyhydroxide is included, a problem may occur in stability of the solution. For example, the insulation coating composition may include 20 to 55 parts by weight of the metal oxyhydroxide.

The metal oxyhydroxide may include at least one of TiOOH, ZrOOH, and MnOOH. For example, it may include at least one of TiOOH and ZrOOH. In some embodiments, it may simultaneously include TiOOH and ZrOOH. If TiOOH and ZrOOH are simultaneously included, it may include 10 to 40 parts by weight of TiOOH and 10 to 40 parts by weight of ZrOOH. For example, it may include 10 to 15 parts by weight of TiOOH and 10 to 40 parts by weight of ZrOOH.

An insulation coating composition for an electrical steel sheet according to an embodiment of the present disclosure may include 0.5 to 10 parts by weight of a reducing agent based on 100 parts by weight of the metal phosphate.

Any reducing agent that may convert the above-described metal oxyhydroxide into an insoluble material by a reduction reaction during a formation process of the coating may be used without limitation.

For example, it may include at least one of ammonia, glycol, polyol, and sulfate. In some embodiments, it may include at least one of ammonia, ethylene glycol, propane-1,2,3-triol, and sodium sulfate.

If there is too little reducing agent, it may be difficult to sufficiently reduce the above-described metal oxyhydroxide. If there is too much reducing agent, it may be gelled in the solution so that a problem occurs in stability of the solution. For example, the insulation coating composition may include 1 to 5 parts by weight of the reducing agent.

In addition to the above-described component, the composition for forming the insulation coating may further include a solvent. The solvent may serve to facilitate application of the composition and uniformly disperse components. An amount of the solvent is not particularly limited, but may be included in an amount of 100 parts by weight to 1000 parts by weight based on 100 parts by weight of the metal phosphate.

FIG. 1 shows a schematic diagram of a cross-section of an electrical steel sheet 100 according to an embodiment of the present disclosure. As shown in FIG. 1, the electrical steel sheet 100 according to the embodiment of the present disclosure may include an electrical steel sheet substrate 10 and an insulation coating 20 disposed on the substrate 10 of the electrical steel sheet.

The electrical steel sheet substrate 10 may use a general non-oriented electrical steel sheet or a general grain-oriented electrical steel sheet without limitation. In an embodiment of the present disclosure, because a main configuration is forming of the insulation coating 20 of a special component on the electrical steel sheet substrate 10, a detailed description of the electrical steel sheet substrate 10 will be omitted.

In addition, a component of the grain-oriented electrical steel sheet substrate is described as follows.

The grain-oriented electrical steel sheet substrate may include 2.0 to 7.0 wt% of silicon (Si), 0.020 to 0.040 wt% of aluminum (Al), 0.01 to 0.20 wt% of manganese (Mn), 0.01 to 0.15 wt% of phosphorus (P), 0.01 wt% or less (excluding 0%) of carbon (C), 0.005 to 0.05 wt% of nitrogen (N), and 0.01 to 0.15 wt% of each of antimony (Sb), tin (Sn), and a combination thereof, and may include the balance of Fe and an inevitable impurity. Because a description of each component of the grain-oriented electrical steel sheet substrate 10 is the same as that generally known, a detailed description thereof will be omitted.

A metal oxide layer (e.g., a base coating layer or a primary coating) formed by reacting an annealing separator with an oxide layer of the steel sheet in a secondary recrystallization process may exist between the grain-oriented electrical steel sheet substrate and the insulation coating. An example of the metal oxide layer may be a forsterite layer. During a manufacturing process of the grain-oriented electrical steel sheet, it is possible to suppress formation of the metal oxide layer or to remove the metal oxide layer so that the grain-oriented electrical steel sheet substrate and the insulation coating are in contact with each other.

A thickness of the insulation coating 20 may be 0.5 to 10 µm. If the thickness of the insulation coating 20 is too small, it may be difficult to secure adequate insulation. If the thickness of the insulation coating 20 is too large, a space factor may be low. In an embodiment of the present disclosure, even if the insulation coating 20 having a thin thickness is formed, an appropriate insulation property may be secured. For example, the thickness of the insulation coating 20 may be 1 to 5 µm.

The insulation coating 20 may include 100 parts by weight of metal phosphate, 25 to 150 parts by weight of silica, 15 to 60 parts by weight of metal oxyhydroxide, and 0.5 to 10 parts by weight of a reducing agent. The insulation coating may be substantially the same as a solid content component within the insulation coating composition described above.

A method for manufacturing the electrical steel sheet according to an embodiment of the present disclosure may include a step of preparing the electrical steel sheet substrate; a step of applying the insulation coating composition to a surface of the electrical steel sheet substrate; and a step of heat-treating the electrical steel sheet substrate.

Because the electrical steel sheet substrate and the insulation coating composition have been described in detail above, a redundant description thereof will be omitted.

For example, the substrate of an electrical steel sheet may be manufactured as follows.

A steel slab may be prepared. Next, the steel slab may be heated. In this case, the slab may be heated using a low-temperature slab method at 1,200°C or less. Next, the heated steel slab may be hot-rolled to manufacture a hot-rolled sheet. Thereafter, the manufactured hot-rolled sheet may be hot-rolled and annealed. Next, the hot-rolled sheet may be cold-rolled to manufacture a cold-rolled sheet. The cold rolling may be performed once, or the cold rolling may be performed two or more times including intermediate annealing. Next, primary recrystallization annealing of the cold-rolled sheet may be performed. In this case, the step of performing primary recrystallization annealing on the cold-rolled sheet may include a step of simultaneously performing decarbonization annealing and nitriding annealing on the cold-rolled sheet, or may include a step of performing nitriding annealing after performing decarbonization annealing. Next, an annealing separator may be applied on a surface of the primary recrystallization-annealed steel sheet. An application amount of the annealing agent may be 1 to 5 g/m². If the application amount of the annealing agent is too small, a coating may not be formed smoothly. If the application amount of the annealing agent is too large, the application amount of the annealing agent may affect the secondary recrystallization. Therefore, the application amount of the annealing agent may be adjusted within the above-described range. Next, secondary recrystallization annealing may be performed on the steel sheet to which the annealing separator is applied. During the secondary recrystallization annealing, a primary cracking temperature may be 650 to 750°C, and a secondary cracking temperature may be 1100 to 1250°C. A temperature condition of the heating section may be controlled at 15°C/hr. In addition, a step to a primary cracking step may be performed in a gas atmosphere including 20 to 30 volume% of nitrogen and 70 to 80 volume% of hydrogen, and a secondary cracking step may be maintained in a 100% hydrogen atmosphere for 15 hours and then furnace cooling may be performed in the secondary cracking step.

In the heat treatment step, a heat treatment temperature may be 700 to 1000°C. If the temperature is too low, a time required to form the insulation coating may be too long so that continuous processing workability is deteriorated. If the temperature is too high, heat resistance and bluing resistance may be reduced due to a crack. For example, the heat treatment temperature may be 750 to 950°C. In some embodiments, it may be 750 to 900°C. The heat treatment time may be from 10 to 300 seconds. For example, it may be 30 to 180 seconds.

An atmosphere during the heat treatment may be a nitrogen atmosphere.

Hereinafter, an embodiment of the present disclosure, a comparative example compared with the embodiment, an evaluation example of the embodiment, and an evaluation example of the comparative example will be described. However, the following embodiment is only the embodiment of the present disclosure, and the present disclosure is not limited to the following embodiment.

### Embodiment

A grain-oriented electrical steel sheet (300mm*60mm) including 3.1% of Si by a weight ratio and having a primary coating with a sheet thickness of 0.23 mm finished annealed is prepared as a test material.

An insulation coating composition is manufactured by mixing components in ratios listed in Table 1 below. First, basic colloidal silica having an average particle diameter of 15 nm and a pH of 10 is introduced in and mixed with a phosphate solution including 50 parts by weight of aluminum phosphate and 50 parts by weight of magnesium phosphate. Thereafter, metal oxyhydroxide and a reducing agent are added to finally manufacture the insulation coating composition.

The manufactured solution is applied on both surfaces of the electrical steel sheet at 3.1 g/mm², and is heat-treated at 850°C for 45 seconds to form an insulation coating with a thickness of 1 µm.

Weather resistance, corrosion resistance, solution stability, and adhesion are evaluated by the following method so that the evaluated results are organized in Table 2.

### Weather resistance evaluation

The weather resistance is evaluated under a condition of 98% moisture, 60 °C, and 72 hours, and if it is good, it is indicated as "OK", and if it is poor, it is indicated as "NG".

### Corrosion resistance evaluation

A salt water spray test of 5% NaCl, 100% RH, 65 °C, and 8 hours is performed. If it is good, it is indicated as "OK", and if it is poor, it is indicated as "NG".

### Solution stability evaluation

After a solution is kept at 30°C for 72 hours, a viscosity thereof is measured using a Brookfield viscometer. If it is less than or equal to 10 cp, it is indicated as "OK", and if it is greater than 10 cp, it is indicated as "NG".

### Adhesion evaluation

In the evaluation of the adhesion, the insulation coating composition is heated for 2 hours under a condition of 560°C, 20% of hydrogen, and 80% of nitrogen. Thereafter, the adhesion is evaluated through a cross-hatch cut test.

If a result of the test is 5B or higher and is good, it is indicated as "OK", and if the result of the test is less than 5B and is poor, it is indicated as "NG".

**(Table 1)**

| Classification (parts by weight) | Phosphate | Silica | d | Ti(OOH) | Reducing agent |
|---|---|---|---|---|---|
| 1 | 100 | 39 | 0 | 0 | 1.32 (ammonia) |
| 2 | 100 | 39 | 26.3 | 13.2 | 1.32 (ethylene glycol) |
| 3 | 100 | 39 | 13.2 | 13.2 | 1.32 (propane-1,2,3-triol) |
| 4 | 100 | 52.6 | 13.2 | 13.2 | 1.32 (sodium sulfate) |
| 5 | 100 | 39 | 26.3 | 0 | 1.32 (ammonia) |
| 6 | 100 | 39 | 13.2 | 0 | 1.32 (ethylene glycol) |
| 7 | 100 | 39 | 52.6 | 0 | 1.32 (propane-1,2,3-triol) |
| 8 | 100 | 39 | 39.5 | 13.2 | 1.32 (sodium sulfate) |
| 9 | 100 | 39 | 0 | 52.6 | 1.32 (ammonia) |
| 10 | 100 | 39 | 0 | 13.2 | 1.32 (ethylene glycol) |
| 11 | 100 | 39 | 0 | 26.3 | 1.32 (propane-1,2,3-triol) |
| 12 | 100 | 39 | 0 | 21.1 | 1.32 (sodium sulfate) |
| 13 | 100 | 39 | 0 | 52.6 | 1.32 (ammonia) |
| 14 | 100 | 39 | 0 | 65.8 | 1.32 (ethylene glycol) |
| 15 | 100 | 74 | 99.5 | 0 | 2.49 (propane-1,2,3-triol) |
| 16 | 100 | 80 | 124.4 | 0 | 2.49 (sodium sulfate) |
| 17 | 100 | 184 | 52.6 | 0 | 1.32 (ammonia) |
| 18 | 100 | 21 | 52.6 | 0 | 1.32 (ethylene glycol) |
| 19 | 100 | 39 | 52.6 | 0 | 0.26 (propane-1,2,3-triol) |
| 20 | 100 | 78 (acidity) | 52.6 | 0 | 13.16 (sodium sulfate) |
| 21 | 100 | 39 | 52.6 | 0 | 0 |
| 22 | 100 | 39 | 13.2 (ZrO₂) | 13.2 (TiO₂) | 1.32 (ammonia) |

**(Table 2)**

| Classification | Weather resistance | Corrosion resistance | Solution stability | Adhesion | |
|---|---|---|---|---|---|
| 1 | NG | NG | OK | OK | Comparative Example |
| 2 | OK | OK | OK | OK | Embodiment |
| 3 | OK | OK | OK | OK | Embodiment |
| 4 | OK | OK | OK | OK | Embodiment |
| 5 | OK | OK | OK | OK | Embodiment |
| 6 | OK | NG | OK | NG | Comparative Example |
| 7 | OK | OK | OK | OK | Embodiment |
| 8 | OK | OK | OK | OK | Embodiment |
| 9 | OK | OK | OK | OK | Embodiment |
| 10 | OK | OK | OK | NG | Comparative Example |
| 11 | OK | OK | OK | OK | Embodiment |
| 12 | OK | OK | OK | OK | Embodiment |
| 13 | OK | OK | OK | OK | Embodiment |
| 14 | OK | OK | NG | OK | Comparative Example |
| 15 | OK | OK | NG | OK | Comparative Example |
| 16 | OK | OK | NG | OK | Comparative Example |
| 17 | OK | OK | NG | OK | Comparative Example |
| 18 | OK | OK | NG | OK | Comparative Example |
| 19 | NG | NG | NG | NG | Comparative Example |
| 20 | OK | OK | NG | OK | Comparative Example |
| 21 | NG | NG | OK | NG | Comparative Example |
| 22 | NG | NG | NG | NG | Comparative Example |

As shown in Table 1 and Table 2, if components of the insulation coating composition are included in an appropriate amount, it may be confirmed that the weather resistance, the corrosion resistance, the solution stability, and the adhesion are simultaneously excellent. If the components of the insulation coating composition are not properly included, it may be confirmed that some of the characteristics are inferior. If a TiO₂ powder and a ZrO₂ powder are added instead of the metal oxyhydroxide, it may be confirmed that the solution stability is inferior due to gelation of the solution.

The present disclosure is not limited to the embodiments, may be manufactured in various different forms, and a person of ordinary skill in the art to which the present disclosure belongs will be able to understand that the present disclosure may be implemented in other specific forms without changing the technical idea or essential feature of the present disclosure. Therefore, it should be understood that the embodiments described above are illustrative and not limited in all respects.

**<Description of symbols>**

| | | | |
|---|---|---|---|
| 100: | electrical steel sheet | 10: | electrical steel sheet substrate |
| 20: | insulation coating | | |

## Claims

1. An insulation coating composition for an electrical steel sheet, comprising:
100 parts by weight of metal phosphate;
25 to 150 parts by weight of silica;
15 to 60 parts by weight of metal oxyhydroxide; and
0.5 to 10 parts by weight of a reducing agent.

2. The insulation coating composition of claim 1, wherein the metal phosphate includes at least one of Mg, Ca, Ba, Sr, Zn, and Al.

3. The insulation coating composition of claim 1, wherein the silica has a pH of 8 to 12.

4. The insulation coating composition of claim 1, wherein the metal oxyhydroxide includes at least one of TiOOH, ZrOOH, and MnOOH.

5. The insulation coating composition of claim 1, wherein the reducing agent includes at least one of ammonia, glycol, polyol, and sulfate.

6. The insulation coating composition of claim 1, wherein the reducing agent includes at least one of ammonia, ethylene glycol, propane-1,2,3-triol, and sodium sulfate.

7. An electrical steel sheet, comprising:
an electrical steel sheet substrate; and
an insulation coating that is disposed on a surface of the electrical steel sheet substrate,
wherein the insulation coating includes 100 parts by weight of metal phosphate, 25 to 150 parts by weight of silica, 15 to 60 parts by weight of metal oxyhydroxide, and 0.5 to 10 parts by weight of a reducing agent.

8. A method for manufacturing an electrical steel sheet, comprising:
preparing an electrical steel sheet substrate;
applying an insulation coating composition to a surface of the electrical steel sheet substrate; and
heat-treating the electrical steel sheet substrate,
wherein the insulation coating composition includes 100 parts by weight of metal phosphate, 25 to 150 parts by weight of silica, 15 to 60 parts by weight of metal oxyhydroxide, and 0.5 to 10 parts by weight of a reducing agent.

9. The method of claim 8, wherein the heat-treating of the electrical steel sheet substrate is performed at a temperature of 750 to 1000°C for 10 to 300 seconds.
